# EUROPEAN PATENT APPLICATION

(11) **EP 0 564 249 A1**
(43) Date of publication of application: **06.10.1993**
(21) Application number: 93302490.3
(22) Date of filing: 30.03.1993
(51) Int. Cl.: F41H 5/04, A41D 31/00

(54) **Impact resistant and impact absorbing laminate**

(30) Priority: 30.03.1992 GB 9206917; 03.08.1992 GB 9216459
(71) Applicant: SPORTS PROTECTION LIMITED, Dunstable, Bedfordshire LU6 3AG (GB)
(72) Inventor: Stanesby, Gerald R., Dunstable, Bedfordshire LU6 2QJ (GB); Bell, Keith M., Dunstable, Bedfordshire LU5 5PA (GB)
(74) Representative: Wain, Christopher Paul

(57) **Abstract**

Cellular viscoelastic material is used in laminates thereof as an impact-resistant material useful not only in body protectors but for a wide variety of other purposes too. In simplest form, the laminates comprise a layer of cellular viscoelastic material (2) bonded directly to a skin (1) of synthetic polymeric material. The laminates may also include other laminae.

## Description

The present invention relates to an impact resistant and impact absorbing laminate and to a method of making it.

It is necessary or desirable for many purposes to be able to provide protection against impact damage, both to resist the impact and to absorb the energy of impact. Certain laminates have been developed for this purpose such as those described in our European patent specification no. 0383895A. These comprise a sheet of flexible polymer material of high impact strength, a layer of low density foamed plastics material, and one or more pieces of high density polyethylene foam sandwiched in between. These laminates are made to the desired shape for their end-use, and are particularly (but not exclusively) useful for body protection for both humans and animals, for example, for protection against sporting injuries such as those obtained in cricket, football and yachting, protection against attack and in particular for protection against motorcycle injuries. For example, the laminates may be formed into shin pads, shoulder pads, arm pads, protective life jackets, body armour, lumbar, back or chest protectors. If so desired, the laminates can be incorporated into items of protective clothing, such as leather motorcycle jackets, at locations where additional body protection may be required.

These laminates are semi-rigid and whilst for certain purposes this presents no problem and can indeed be an advantage, in other circumstances the rigidity does detract from the product. For example, there are occasions when the rigid laminate may itself snap or break and it may then aggravate any injury received. Furthermore, rigidity of such protective laminates, especially when they are used to protect knees, elbows etc. can restrict movement. There is therefore a need for protective laminates which do not cause harm should they become damaged, and can be made flexible enough to allow reasonable movement.

Whilst the laminates of our European specification no. 0383895A provide good impact resistance and also good impact energy absorption, we have now found that much better energy absorption can be achieved, with flexibility if desired and with other advantages, by using a different material in the laminates. In particular, we have found that the use in laminates of a sheet of cellular viscoelastic material provides surprisingly good results.

In accordance with one aspect of the present invention, there is provided an impact resistant laminate which comprises bonded therein a sheet of synthetic polymeric material or metal, and a sheet of cellular viscoelastic material.

Cellular viscoelastic materials are known and can be made of rubber itself or other rubber-like materials. They include, for example, rubber-based materials such as Noene or Norsorex (polynorbornene) and Compound 1910 from Volcrepe. These materials have a relatively high loading of carbon and are relatively tear-resistant. Generally, they have an elongation to break of at least about 200%; a density of 700 to 800 kg/m³; and a compression deflection at 25% of 170-210 kPa. In sheet form, cellular viscoelastic materials on their own do not provide much impact resistance or impact energy absorbance. They suffer local flattening in the area of impact, and on their own, they are not particularly useful materials for impact protection. However, when in a laminate, especially with a non-elastic material such as a polyethylene or polypropylene sheet, the cellular viscoelastic material confers surprisingly good energy absorbance on the laminate.

In one arrangement of the present invention, the laminate comprises a skin and a sheet of the cellular viscoelastic material, the skin and the sheet being laminated to each other in such a way that bonding occurs over part or the entirety of their facing surfaces to lock them together, thus effectively limiting the stretchability (elasticity) of said sheet in the bonded areas to correspond to the lower elasticity of said skin, thereby preventing said sheet of viscoelastic material from being pulled thin upon impact.

In these laminates, the skin is normally a sheet of flexible synthetic polymeric material of high impact strength such as low density polyurethane. Other possibilities include high and low density polyethylene or polypropylene, or a sheet of metal.

The laminates of the invention can include other materials such as other layers bonded into the laminate, between the cellular viscoelastic material and the synthetic polymeric sheet or metal skin or outside either or both. Such other layers may include further layers of a cellular viscoelastic material, or of a synthetic polymeric sheet or metal, or both. For example, extra sheets of cellular viscoelastic material laminated to the main sheet of viscoelastic material result in improved impact absorption. Similarly, one or more sheets of cellular viscoelastic material can be sandwiched between two skins, giving the laminate smooth upper and lower surfaces. If buoyancy is required, such as in protective life-jackets, a layer or part layer of very low density closed cell foam may be included in the laminate. A further example would be a laminate including a layer of Kevlar.

In a preferred aspect of the invention, the laminates comprise an outer skin which is impact resistant and semi-rigid, and a layer of the cellular viscoelastic material protected against direct contact with the impact by (at least) the outer skin. Where the laminate comprises several laminae, provision can be made to accommodate some limited lateral slip between adjacent laminae, which can be of advantage in certain situations.

The laminates of the invention may be made by ordinary methods. The cellular viscoelastic layers are usually bondable directly (with heat and pressure) to synthetic polymeric material skins such as polyurethanes or polyolefines. Typical laminating conditions are 110° to 120°C for about 2 minutes under a vacuum blanket pressure of 0.2 bar. The laminate can be shaped at 80° to 160°C for about 2 minutes with a vacuum blanket pressure of 0.4 bar.

Embodiments of the present invention will now be more particularly described by way of example only with reference to the accompanying drawings, wherein:
Figure 1 shows a shin pad embodying the invention;
Figure 2 is a cross-section through a median portion of the shin pad of Figure 1;
Figure 3 is a plan view of a horse cushion of the invention;
Figure 4 is a section on the line 4-4 of Figure 3;
Figure 5 is a front elevation of a protective garment such as a vest, with a trauma pack;
Figure 6 is a section on line 6-6 of the trauma pack of Figure 5; and
Figures 7 (a) - (d) illustrate in section other examples of laminates of the invention.

Referring now to the drawings, and in particular to Figure 2, there is shown a cross-section of a laminate according to the present invention. An outer skin 1 comprises a flexible synthetic polymer material such as low density polyurethane, high or low density polyethylene or polypropylene. The preferred skin 1 is made from low density polyurethane. An inner sheet 2 of cellular viscoelastic material is preferably made from Norsorex or compound 1910. Both Norsorex and compound 1910 have been found to possess superior impact absorbing qualities as well as superior tear resistance. In impact tests one sheet of Norsorex or compound 1910 was found to provide a higher degree of protection against impact damage than six or more equivalent sheets of other protective materials. The density of compound 1910 is approximately 750kg/m³. The laminate is produced in a vacuum mould by placing a sheet of the cellular viscoelastic material 2 onto a layer of skin 1. The assembly is then placed on a flat platen and heated to 110° to 200°C, depending on what materials are used for layers 1 and 2. The laminate is formed after about 2 minutes at a vacuum blanket pressure of 0.2 bar, whereby the sheet of cellular viscoelastic material 2 is bonded to skin 1. Bonding occurs along the entire interface 3 and in this way sheet 2 can now only spread sideways to the same limited extent as skin 1, thus preventing thinning of viscoelastic material 2 upon impact. During the process of lamination care has to be taken at all times not to stretch viscoelastic material 2.

The laminate so formed may then be moulded into the required shape, for example a shin pad, in an epoxy vacuum mould.

Although the present invention has been described with respect to body protectors, the laminates of the present invention have many other applications, for example, as car bumpers, car bonnets and the like.

One very important further such use is in connection with animals, especially horses and ponies which are shod with horseshoes. We have found that it is highly advantageous to provide, between the hoof and the shoe, a laminate of the invention to cushion shock. Preferably, the laminates comprise two polymeric skins of LDP or the like, and a layer of the cellular viscoelastic material therebetween. Conveniently, such laminates are provided in unit form ready for use, to be sandwiched between a horseshoe and the underlying hoof. Spare material projecting laterally of the hoof/shoe is then removed after the shodding.

The accompanying Figure 3 shows in plan view one example of a horse cushion of the invention. It consists of a horseshoe-shaped piece of viscoelastic material (10), wider than the horseshoe, and laminated between two skins (11,12). In use, the cushion is placed between a shoe and the hoof during shodding, and is held in place by the nails used to fix the horseshoe. Any spare cushion material extending laterally is then trimmed off. Figure 4 is a section on line 4-4 of Figure 3. As can be seen, in the central region "inside" the viscoelastic horseshoe the two skins (11,12) are joined directly together, as they are around the outer periphery of the viscoelastic shape 10.

Referring now to Figures 5 and 6, there is shown in Figure 5 a schematic view of a body protector 50, eg. a vest. This will conventionally be made of protective materials, eg. it may include layers of penetration-resisting aramid fabric (eg. Kevlar). It is known to provide such body protectors with a trauma pack 51 which is an extra item of protection securable to the vest at a critical region 52 (eg. over the heart). The trauma pack is especially designed to absorb impact. One example is shown in U.S. 4774724. In accordance with a feature of the present invention, the trauma pack is made of a laminate 53 of the invention. One example is shown in Figure 6: it consists of a front skin layer 54 of low density polyethylene, for example; a layer 55 of polycarbonate or like impact absorbing plastics material; and a layer 56 of viscoelastic material bonded to the polycarbonate. The laminate may include other layers as desired. The whole may be included in a flexible container for attachment to the body protector.

Laminates of the invention are particularly useful in body protectors of various sorts as will be clear to those skilled in the art.

Figures 7(a) - (d) illustrate other laminates of the invention (in section). Figure 7(a) shows a simple arrangement of viscoelastic layer 70 bonded on both major faces to a semi-rigid skin layer 71. In Figure 7(b), the viscoelastic material layer 70 is bonded to an impact resisting layer 72 such as polycarbonate, and the whole is bonded within a skin 73 which can be flexible or semi-rigid, as desired. In Figure 7(c), the laminate has a polycarbonate sheet 80 bonded to one face of the viscoelastic layer 70, and a thin skin 81 eg. of polyethylene is bonded to the other face of the viscoelastic layer 70. A further sheet of material 82 lies next to layer 81 but is not bonded thereto. Sheet 82 is however bonded to outer skin 71. This arrangement allows some limited slip between sheets 81 and 82. Figure 7(d) is similar to Figure 7(b) so far as skin 73 and layers 70 and 72 are concerned. However, a region of aramid fabric 90 is also included, to provide extra penetration resistance. The fabric 90 can be bonded in to the laminate or it may be sandwiched without bonding.

## Claims

1. An impact resistant laminate which comprises bonded therein a sheet of synthetic polymeric material or of metal, and a sheet of cellular viscoelastic material.

2. A laminate according to claim 1, wherein the sheet of viscoelastic material is bonded in the laminate at least over substantially the entirety of one major surface of the sheet.

3. A laminate according to claim 1 or 2, which includes an outer skin of metal or of flexible synthetic polymeric material.

4. A laminate according to claim 3, wherein the skin is of low density polyurethane, or high or low density polyethylene or polypropylene.

5. A laminate according to any of claims 1 to 4, with more than one sheet of viscoelastic material bonded therein.

6. A laminate according to any of claims 1 to 5, wherein the or at least one of the sheets of viscoelastic material is bonded to a sheet of impact resistant material.

7. A laminate according to claim 6, wherein the sheet of impact resistant material is polycarbonate.

8. A laminate according to any of claims 1 to 7, which includes three or more laminae and wherein limited lateral slip is possible between a pair of adjacent laminae.

9. A protective article which comprises an impact resistant laminate as claimed in any preceding claim.

10. A trauma pack for use with personal body protection which comprises a laminate comprising at least a sheet of impact resistant material bonded on one major face to an outer skin of synthetic polymeric material, and on the other major face to a sheet of cellular viscoelastic material.
